

No. 741,494.

PATENTED OCT. 13, 1903.

H. K. HITCHCOCK.  
ANNEALING GLASS SHEETS OR PLATES.

APPLICATION FILED JULY 30, 1902.

NO MODEL.

2 SHEETS—SHEET 1.



WITNESSES:

Herbert Bradley.  
Fred Kirchner.

INVENTOR

Halbert K. Hitchcock  
by Dennis S. Wolcott, Atty.

No. 741,494.

PATENTED OCT. 13, 1903.

H. K. HITCHCOCK.

ANNEALING GLASS SHEETS OR PLATES.

APPLICATION FILED JULY 30, 1902.

NO MODEL.

2 SHEETS—SHEET 2.

FIG. 2.



FIG. 3.



WITNESSES : 3.

*Herbert Bradley.*

*Fred Kirchner.*

INVENTOR

*Herbert K. Hitchcock*  
*by Dennis S. Wolcott* At't'y.

## UNITED STATES PATENT OFFICE.

HALBERT K. HITCHCOCK, OF WALTON, PENNSYLVANIA.

## ANNEALING GLASS SHEETS OR PLATES.

SPECIFICATION forming part of Letters Patent No. 741,494, dated October 13, 1903.

Application filed July 30, 1902. Serial No. 117,639. (No specimens.)

*To all whom it may concern:*

Be it known that I, HALBERT K. HITCHCOCK, a citizen of the United States, residing at Walton, in the county of Allegheny and State of Pennsylvania, have invented or discovered certain new and useful Improvements in Annealing Glass Sheets or Plates, of which improvements the following is a specification.

It has been found in annealing sheets or plates of glass that the edges cool more rapidly than other parts and that the contraction of the edges will produce wave-like surfaces, thereby necessitating long-continued grinding to produce even plane surfaces.

The object of the invention described herein is to provide for a substantially uniform cooling of the entire plate or sheet, thereby avoiding irregularities incident to irregular cooling and contraction.

The invention is hereinafter more fully described and claimed.

In the accompanying drawings, forming a part of this specification, Figure 1 is a plan view of a furnace adapted to the practice of my invention. Figs. 2 and 3 are sectional elevations on planes indicated by the lines II II and III III, Fig. 1; and Fig. 4 is a view in the nature of a diagram illustrative of my invention.

In the practice of my invention the annealing leir or kiln is provided with suitable means whereby the loss of heat by radiation from different portions of the sheet or plate in the kiln can be controlled. A convenient manner for effecting such control is shown in the drawings and consists in providing suitable means for applying a regulated heat to different portions of the compartments 1 of the leir or kiln. This application of heat can be effected by providing heating-chambers 2, 3, and 4 outside of the walls proper of the compartments. The chambers are provided with suitable outlets, so that there may be a circulation of the heat through such chambers, and it is preferred that each heating-chamber should have independent heat-generators. As shown in the drawings, the chambers 2 under the floors of the annealing-compartments are connected by flues 5 with a stack 6, and burners 7 from the supply-pipes 8 extend up into said chambers. These burners are preferably arranged in or approxi-

mately in line with the edges of the sheets or plates when in position in the compartments, and the flues 6 connect with the heating-chambers at a point approximately central of the burners. The side chambers 3 connect with the top chambers 4, which are provided with outlet-flues 9. Burners 10 extend from the supply-pipes 8 into the side chambers 3 near their lower portions, and the heat therefrom flows up into the top chambers. As the initial or charging compartment has heating-chambers on three sides only and the other compartments on only two sides, (said heating-chambers being arranged in the outer walls of said compartments,) portions of the upper chambers might not be sufficiently heated from the side chambers. Uniform heating of the top chambers is attained by means of burners 11, extending into the portions of the top chambers not in the line of flow of heat from the side chambers.

The curtain-walls 13, separating the compartments, are made hollow, as shown, and connect at the ends with the side chambers 3, so that said walls will receive some heat from the side chambers.

It will be readily understood by those skilled in the art that other means may be employed for maintaining any desired heat in any portion of each compartment, and hence the broader claims are not limited to any specific means for applying heat to the sheets or plates in the leir or kiln.

It is characteristic of my improvement that by the proper regulation of the heating devices the cooling down, and consequent contraction, of the sheets or plates can be made uniform throughout, thus avoiding any distortion of parts by the prior cooling and contraction of other parts. It will be understood that each compartment is maintained at a lower temperature than the preceding compartment. If the edges of the sheet or plate are too cool when charged into the leir, such edges may be heated up by increasing the heat in the bottom and side chambers.

In Fig. 4 is shown a portion of a plate of glass. As the portion of the plate outside of the line *a c*, having a radiating-surface represented by the line *a b c*, will contain less heat units than the portion between the lines *a c* and *d e*, the radiating-surface of such por-

tion being represented by the line  $a\ d$  and equal to the surface  $a\ b\ c$ , it follows that the latter portion will cool more slowly than the edge portion  $a\ b\ c$ . Hence to prevent the 5 more rapid cooling of the edge portion the radiation therefrom is reduced or checked by the proper regulation of the heat-generators, as described. In case the edges have become comparatively cool before the sheet or 10 plate is stowed in the kiln or leer, by increasing the heat at the edges of the sheet or plate they may be rendered sufficiently plastic to allow the wrinkles or waves in the body portion to flatten out.

15 While I have shown and described with some particularity an apparatus adapted to the practice of my invention, the claims herein are not limited to the employment of such 20 specific form of apparatus, which forms no part of the subject-matter of this application.

I claim herein as my invention—

1. An improvement in the art of annealing

sheets or plates of glass, which consists in bringing all portions of the sheet or plate to a uniform or approximately uniform temperature and then so regulating the radiation of heat units that the cooling of the sheet or plate shall be equal in all parts, substantially as set forth. 25

2. As an improvement in the art of annealing sheets or plates of glass, the method herein described which consists in so regulating the radiation and consequent cooling of the edges of the sheets of glass that the contraction along such edges will be approximately 30 simultaneous and uniform with the contraction of other portions, substantially as set forth. 35

In testimony whereof I have hereunto set my hand.

HALBERT K. HITCHCOCK.

Witnesses:

DARWIN S. WOLCOTT,  
F. E. GAITHER.